

## UNITED STATES PATENT OFFICE.

NATHANIEL C. FOWLER, OF BOSTON, MASSACHUSETTS, ASSIGNOR, BY MESNE ASSIGNMENTS, TO THE INDESTRUCTIBLE SAFE AND FIRE PROOF COMPANY, OF WEST VIRGINIA.

## FIRE-PROOF COMPOUND AND SHEET.

SPECIFICATION forming part of Letters Patent No. 288,935, dated November 20, 1883.

Application filed June 28, 1883. (Specimens.)

*To all whom it may concern:*

Be it known that I, NATHANIEL C. FOWLER, of Boston, in the county of Suffolk and State of Massachusetts, have invented a new and useful Improvement in Fire-Proof Compounds and Sheets made thereof, which invention I will describe as follows:

My invention consists in a mechanically-mixed compound in a dry state, composed of the following articles, the proportions of which will be hereinafter fully given, viz: calcined plaster-of-paris, (gypsum,) asbestos finely fibrilized, lamp-black, and finely-ground pumice-stone. The proportions are to be taken by relative bulk or cubic measurement, and not by weight.

The invention also consists in rendering the mixture sufficiently consistent by means of wafer, and then running the mass off onto a table or other suitable surface in as thick sheets and of the size required. When these sheets are dry, they may be used in the construction of fire-proof boxes, for the lining of fire-proof safes, or for other like purposes.

The proportions for the mixture should be ascertained as above described, and should be substantially as follows: about seventy per centum of calcined plaster-of-paris, about twenty per centum of asbestos, five per centum (more or less) of lamp-black, and about five per centum of pumice-stone.

Though asbestos is fire-proof, its principal value in this compound consists in its adhesive quality. Being, as it is, a fibrous material, it gives strength to the entire mass, and prevents the crumbling which might come from jarring or other causes.

Lamp-black is combustible when subjected to a high degree of heat; but is of value in this compound because of the fact that when evenly and carefully mixed therewith it renders the whole mass porous, and it is a well-known fact that an infinite number of air-cells increases very largely the capacity of a fabric to resist the action of heat.

Other articles—such as finely-ground saw-

dust or wood pulp—could be used; but lamp-black is preferable because of its infinite fineness, and thus its usefulness in producing an infinite number of air-cells. A larger proportion of lamp-black than five per cent. could be used; but as this material may be destroyed by a high temperature, as I have stated, it is better that not more than about five per cent. of the entire bulk be employed, for were this moderate percentage of lamp-black to be destroyed, the capacity of the rest of the mass to successfully resist the action of heat would not be materially lessened.

Sheets may be produced as above described, and they may be jointed one to another by moistening their edges with water—preferably warm water.

While the mass is in a plastic state it can be molded into any shape desired, or it may be filled into the hollow sides of a safe or box.

Having thus fully described my invention and the manner of carrying the same into effect, what I claim as new, and desire to secure by Letters Patent, is—

1. In combination, calcined plaster-of-paris, finely-fibrilized asbestos, lamp-black, and finely-ground pumice-stone, the whole compounded in a dry state, and in substantially the proportions described, said proportions to be ascertained upon the basis of bulk, substantially as described.

2. As an article of manufacture, sheets of fire-proof material produced by compounding, when in a dry state, calcined plaster-of-paris, finely-fibrilized asbestos, lamp-black, and pumice-stone, in substantially the proportions and in the manner described, such dry compound to be wet with water to a suitable consistency, then run off upon a level surface into the thickness and size of sheets desired, and allowed to dry, all substantially as described.

NATHANIEL CLARKE FOWLER.

Witnesses:

FRANCIS W. BOUTWELL,  
FLORENCE L. EMERY.